# EUROPEAN PATENT SPECIFICATION

(11) **EP 0 083 842 B1**
(45) Date of publication and mention of the grant of the patent: **12.07.1989**
(21) Application number: 82306473.8
(22) Date of filing: 06.12.1982
(51) Int. Cl.: C22C 29/00, B22F 7/04, C23C 16/30

(54) **Surface-coated hard metal body and method of producing the same**
Beschichteter Hartmetallkörper und Verfahren zu seiner Herstellung
Elément en métal dur revêtu et procédé de sa fabrication

(30) Priority: 16.12.1981 US 331367; 16.12.1981 US 331368
(43) Date of publication of application: 20.07.1983
(73) Proprietor: CARBOLOY INC., Warren Michigan 48089-3071 (US)
(72) Inventor: Hale, Thomas Eugene, Warren Michigan 48093 (US)
(74) Representative: Turner, Paul Malcolm

(56) References cited:
- EP-A- 0 032 887
- US-A- 4 018 631
- US-A- 4 019 873
- US-E- 29 420
- PATENT ABSTRACTS OF JAPAN, unexamined applications, field C, vol. 5, no. 28, February 20, 1981 THE PATENT OFFICE JAPANESE GOVERNMENT page 122 C 44
- PATENT ABSTRACTS OF JAPAN, unexamined applications, field C, vol. 4, no. 178, December 10, 1980 THE PATENT OFFICE JAPANESE GOVERNMENT page 116 C 34

## Description

This invention relates to coated articles comprising hard metals, refractories, and especially cemented carbide substrates. More particularly, it relates to such coated hard metal or coated cemented carbide products which are adapted to receive an aluminum oxide or other oxide wear layer which is very firmly bonded to the substrate.

Such hard metal and/or cemented carbide substrates are used in tools for machining and cutting metals. Their already high wear resistance can be significantly improved by providing oxide wear layers, such as aluminum oxide wear layers, as described in U.S. 3,736,107 and 3,836,392. However, it has become apparent that proper steps must be taken to adequately bond the oxide layer to the hard metal or cemented carbide substrate if the superior wear resistance of the oxide layer is to be realized.

In U.S. 4,018,631, it is disclosed that a selective pretreatment of cemented carbides before application of the oxide wear layer unexpectedly enhances and improves the adherence of the subsequently applied oxide wear layer. While such a procedure results in a tightly adherent surface layer of aluminum oxide or other oxide wear layer, and is therefore extremely useful, the procedure requires a high temperature for the diffusion step.

A novel coating procedure has now been discovered which provides aluminum oxide and other oxides (e.g., hafnium oxide, zirconium oxide and the like) bonded to the substrates with adherence equal to that obtained in the said '631 patent, which can be performed at normal coating temperatures.

The present bonding layer is thin, not useful as a barrier, and possesses a composition novel in its chemical constituents. All of the foregoing patents and publications are incorporated herein by reference.

According to the invention there is provided an article for cutting and wear parts comprising:
(i) a hard metal or cemented carbide substrate;
(ii) a first coating on the substrate of a carbide, nitride, or carbonitride, of titanium, zirconium, hafnium, vanadium, niobium, tantalum, chromium, molybdenum, tungsten, silicon or boron;
(iii) a bonding layer attached to said first coating, the bonding layer being a surface-oxidized bonding layer comprising at least one of the carbides or oxycarbides of tantalum, niobium and vanadium and including aluminium, said bonding layer being capable of adherently accepting an oxide wear layer at coating temperatures of from 800°C to 1300°C; and
(iv) an oxide wear layer overlying said bonding layer.

The present invention also provides a process of pretreating a hard metal or cemented carbide substrate for the reception of wear resistant oxide coatings which comprises:
(a) applying a first coating to the substrate of a carbide, nitride or carbonitride, of titanium, zirconium, hafnium, vanadium, niobium, tantalum, chromium molybdenum, tungsten, silicon or boron;
(b) treating the coated substrate in a first atmosphere selected from carbide and oxycarbide forming atmospheres to form a bonding layer of a carbide or oxycarbide of a metal selected from at least one of tantalum, niobium or vanadium on said coated substrate;
(c) heating the coated substrate of (b) at a temperature of from 800° to 1300°C in a further oxidizing atmosphere until at least portions of the surface are oxidized; and
(d) treating the oxidized coated substrate of (c) in a reducing atmosphere with a reducible aluminium compound to diffuse aluminium into the coating.

In preferred features, the substrate is a cobalt cemented carbide; the bonding layer is 0.1 to 0.5 pm thick; the oxide wear layer is aluminium oxide; and the wear layer is 0.5 to 20 pm thick.

In one practice of the present invention a hard metal or cemented carbide substrate is precoated with a layer comprising a carbide, nitride or carbonitride of Ti, Zr, Hf, V, Nb, Ta, Cr, Mo, W, Si or B to form an intermediate layer, the preferred layer being TiC. The substrate is then treated in a first atmosphere selected from carbide and oxycarbide forming atmospheres to form a bonding layer of a metal selected from at least one of tantalum, niobium or vanadium on said coated substrate and heating the coated substrate in a second oxidizing atmosphere until at least about 50% of the surface is oxidized.

Aluminium is added to the bonding layer; and an oxide outer wear layer, preferably an aluminium oxide wear layer, will be deposited on the bonding layer.

Those skilled in this art will know the general techniques used to prepare the product and carry out the process of the present invention.

One convenient way of proceeding is to provide a coating furnace held at a temperature of from about 800°C to 1300°C, and to expose a precoated substrate of the process of step (a) in the furnace to the following sequential steps.
1. 5 to 60 minutes exposure, preferably at 1050°C, to a gaseous mixture of H₂ and 0.5 to 20 volumes percent TaCI₅ or NbClₛ; TiCl₄, AIC1₃ and/ or CH₄ may be optionally added during either part or all of this period.
2. 1 to 60 minutes exposure, preferably at 1100°C, to a gaseous mixture consisting of H₂ and about 1 to 50 volume percent C0₂ to oxidize and produce the pretreated substrate.
3. 5 to 60 minutes exposure, preferably at 1050°C, to a gaseous mixture of H₂ and about 0.5 to 20 volume percent AICI₃. This is the step for adding aluminium.
4. 15 minutes' to 4 hours' exposure, preferably at 1050°C, to a gaseous mixture of H₂, 1 to 40 (or 60 to 95) volume percent C0₂, and 2.5 to 20 volume percent AIC1₃ to produce the aluminium oxide wear coating.

Other suitable treating atmospheres of varying proportions of constituents will occur to those skilled in the art. Likewise, other well known deposition techniques can be used such as physical vapor deposition, sputtering and pack diffusion.

Those features of the invention which are believed to be novel are set forth with particularity in the claims appended hereto. The invention will, however, be better understood from a consideration of the preferred embodiments.

The following examples are illustrative, and the claims are not be construed as being limited thereto.

### Example 1

A commercial cemented carbide cutting tool insert of composition 85.5% WC, 6% TaC, 2.5% TiC and 6% Co was coated in the following manner:
1. Held 15 minutes at 1050°C in an atmosphere of H₂―5% CH₄―2% TiCl₄―5% TaCl₅―10% AICI₃.
2. Held 40 minutes at 1050°C in an atmosphere of H₂-10% C0₂.
3. Held 10 minutes at 1050°C in an atmosphere of H₂―10% AlCl₃.
4. Held 60 minutes at 1050°C in an atmosphere of H₂―10% CO₂―10% AlCl₃.

This treatment resulted in a 4 µm Al₂O₃ coating which was firmly bonded to the cemented carbide substrate through a bonding layer about 0.2 pm thick.

The coated insert was used to machine cast iron at 122.1 surface metres per minute, 0.025 mm/rev. feed rate, and the wear resistance was compared with that obtained using a commercial insert which requires a high temperature diffusion operation to make the coating.

The wear resistance of the insert coated by the above-described simplified process was found to be nearly equal to that of the commercial insert.

### Example 2

A cemented carbide insert having the same composition as Example 1 above was coated with Al₂O₃ in the following manner:
1. Held 15 minutes at 1050°C in a gaseous mixture of H_{2―}2% TiC₄―5% NbCi₅―10% AlCl₃ₐ, then the TiCf₄ was turned off and the insert was held an additional 10 minutes at 1050°C in the remaining mixture of H₂―5% NbCl₅ 10% AlCl₃.
2. Held 20 minutes at 1100°C in a mixture of H₂―5% CO₂.
3. Held 20 minutes at 1050°C in a mixture of H₂-10% AICI₃.
4. Held 45 minutes at 1050°C in a mixture of H_{2―}5% CO₂―10% AlCl₃.

The resultant coated insert had a 3 µm Al₂O₃ coating firmly bonded to the cemented carbide substrate, through a bonding layer about 0.2 pm thick attached to a carbide layer formed from the niobium and titanium and carbon from the substrate.

When used to machine cast iron (same conditions as Example 1 above), the wear resistance was found to be equivalent to the commercial insert.

### Example 3

A cemented carbide insert having the same composition as Example 1 above was pretreated then coated with Al₂O₃ in the following manner at a furnace temperature of 1050°C, and 10⁵ Pa (1 atmosphere) pressure.
1. Held 10 minutes in a gaseous mixture of H₂―10% CH₄.
2. Held 1 minute in a gaseous mixture of H₂―2% TiCl₄.
3. Held 25 minutes in a mixture of H₂ and NbCl (which had been heated for about 8 minutes to 160°C., held 3 minutes, and cooled with power off for 15 minutes).

Steps 1 to 3 produce a carbide and bonding layer.
4. Held 2 minutes in a gaseous mixture of H₂―2.5% CO₂.
5. Held 10 minutes in a gaseous mixture of H₂―5% AliCl₃.
6. Held 60 minutes in a gaseous mixture of H₂―5% AlCl₃-9% CO₂.

The resultant coated insert had a 3-4 µm A₂l₂O₃ coating firmly bonded to the cemented carbide substrate, through a bonding layer about 0.2 µm thick.

When used to machine cast iron (same conditions as Example 1 above), the wear resistance is found to be equivalent to the commercial insert.

### Example 4

The procedure of Example 3 was repeated, using the following conditions:
1. Held 1 minute at 1050°C in a gaseous mixture of H₂-3% TiCl₄.
2. Held 1 minute at 1050°C in a gaseous mixture of H₂-3% TiCl₄―20% N₂.
3. Held 30 minutes in H₂―3% NbCl₅;+3% TiCl₄ added for 20 seconds during middle of this period and temperature was 850°C for first 10 minutes of this period and then increased in a linear fashion to 1050°C by the end of the period.

Steps 1 to 3 produce a carbide and a bonding layer, the carbon being derived from the substrate.
4. Held 10 minutes at 1050°C in H₂―11% CO₂.
5. Held 10 minutes at 1050°C in H₂-7% AlCl₃.
6. Held 60 minutes in gaseous mixture of H₂―11% CO₂ 7% AlCl₃.

A coated insert according to this invention was obtained.

### Example 5

A commercial cemented carbide cutting tool insert comprising 85.5% WC, 6% TaC 2.5% TiC and 6% Co and coated with TiC of five µm thickness is subjected to the following sequence of steps in a furnace at temperature of 1050°C and 10⁵ Pa (1 atmosphere) pressure:
1. 2 minutes in an atmosphere of H₂ and approximately 2% TiCl₄.
2. NbClₛ vaporizer on 8 min. to 107°C., 3 min. hold-15 min. power off-cool.
   Steps 1 and 2 produce a carbide and a bonding layer using carbon from the substrate.
   3. 1 minute in an atmosphere of hydrogen-3.5% C0₂ to surface oxidize.
   4. 10 minutes in an atmosphere of hydrogen-5% AICI₃.
   5. 60 minutes in an atmosphere of hydrogen-5% AlCl₃-7% CO₂.

This treatment resulted in a 3-4 pm A1₂0₃ coating which was firmly bonded to the TiC coated cemented carbide substrate, through a bonding layer approximately 0.2 pm thick.

The coating adhesion of this insert was sufficient to meet the requirements of commercial A1₂0₃-coated substrates, without a TiC layer. Direct deposit of A1₂0₃ on inserts coated with TiC fail to meet these requirements.

## Claims

1. An article for cutting and wear parts comprising:
(i) a hard metal or cemented carbide substrate;
(ii) a first coating on the substrate of a carbide, nitride, or carbonitride, of titanium, zirconium, hafnium, vanadium, niobium, tantalum, chromium, molybdenum, tungsten, silicon or boron;
(iii) a bonding layer attached to said first coating, the bonding layer being a surface-oxidized bonding layer comprising at least one of the carbides of oxycarbides of tantalum, niobium and vanadium and including aluminium said bonding layer being capable of adherently accepting an oxide wear layer at coating temperatures of from 800° to 1300°C; and
(iv) an oxide wear layer overlying said bonding layer.

2. An article as claimed in Claim 1 wherein said first coating comprises TiC.

3. A process of pretreating a hard metal or cemented carbide substrate for the reception of wear resistant oxide coatings which comprises:
(a) applying a first coating to the substrate of a carbide, nitride or carbonitride, of titanium, zirconium, hafnium, vanadium, niobium, tantalum, chromium, molybdenum, tungsten, silicion or boron;
(b) treating the coated substrate in a first atmosphere selected from carbide and oxycarbide forming atmospheres to form a bonding layer of a carbide or oxycarbide of a metal selected from at least one of tantalum, niobium or vanadium on said coated substrate;
(c) heating the coated substrate of (b) at a temperature of from 800° to 1300° in a further oxidizing atmosphere until at least portions of the surface are oxidized; and
(d) treating the oxidized coated substrate of (c) in a reducing atmosphere with a reducible aluminium compound to diffuse aluminium into the coating.

4. A process as claimed in Claim 3 including the step of superimposing an oxide wear layer on the surface-oxidized, aluminium-containing coated substrate.

## Patentansprüche

1. Gegenstand für Scheide- und Verschleißteile, der umfaßt:
(i) ein Substrat aus Hartmetall oder Sinterhartmetall;
(ii) eine erste Beschichtung auf dem Substrat aus einem Carbid, Nitrid oder Carbonitrid von Titan, Zirkon, Hafnium, Vanadium, Niob, Tantal, Chrom, Molybdän, Wolfram, Silicium oder Bor;
(iii) eine auf der ersten Beschichtung aufgebrachte Bindungsschicht, wobei die Bindungsschicht eine obereflächenoxidierte Bindungsschicht ist, die mindestens eines der Carbide oder Oxycarbide von Tantal, Niob und Vanadium umfaßt und Aluminium enthält, und wobei die Bindungsschicht zur festhaftenden Aufnahme einer Oxid-Verschleißschicht bei Beschichtungstemperaturen von 800° bis 1300°C geeignet ist; und
(iv) eine die Bindungsschicht bedeckende Oxid-Verschleißschicht.

2. Gegenstand nach Anspruch 1, in dem die erste Beschichtung TiC umfaßt.

3. Verfahren zur Vorbehandlung eines Substrates aus einem Hartmetall oder Sinterhartmetall für die Aufnahme von verschleißfesten Oxidbeschichtungen, das umfaßt:
(a) Aufbringen einer ersten Beschichtung auf das Substrat aus einem Carbid, Nitrid oder Carbonitrid von Titan, Zirkon, Hafnium, Vanadium, Niob, Tantal, Chrom, Molybdän, Wolfram, Silicium oder Bor;
(b) Behandeln des beschichteten Substrates in einer ersten Atmosphäre, die ausgewählt ist aus Carbid- und Oxycarbid-erzeugenden Atmosphären, zur Erzeugung einer Bindungsschicht aus einem Carbid oder Oxycarbid mindestens eines der Metalle Tantal, Niob oder Vanadium auf dem beschichteten Substrat;
(c) Erhitzen des beschichteten Substrates von (b) auf eine Temperatur von 800° bis 1300°C in einer weiteren oxidierenden Atmosphäre, bis zumindest Teile der Oberfläche oxidiert sind; und
(d) Behandeln des oxidierten, beschichteten Substrats von (c) in einer reduzierenden Atmosphäre, mit einer reduzierbaren Aluminiumverbindung, um Aluminium in die Beschichtung einzudiffundieren.

4. Verfahren nach Anspruch 3, das die Stufe der Überschichtung des oberflächenoxidierten, Aluminium enthaltenden beschichteten Substrates mit einer Oxid-Verschleißschicht einschließt.

## Revendications

1. Article pour élément de coupe et d'usure, comprenant:
(i) un substrat en métal dur ou carbure cémenté;
(ii) un premier revêtement, sur ce substrat, en un carbure, nitrure ou carboniture de titane, zirconium, hafnium, vanadium, niobium, tantale, chrome, molybdène, tungstène silicium ou bore;
(iii) une couche de liaison, fixée audit premier revêtement, cette couche de liaison étant une couche de liaison oxydée en surface et comprenant au moins un des carbures ou oxycarbures de tantale, niobium, et vanadium, et comprenant de l'aluminium, ladite couche de liaison étant capable d'accepter, de façon adhésive, une couche d'usure en oxyde, à des températures de revêtement de 800° à 1300°C; et
(iv) une couche d'usure en oxyde, superposée à ladite couche de liaison.

2. Article tel que revendiqué dans la revendication 1, dans lequel ledit premier revêtement comprend TiC.

3. Procédé de prétraitment d'un substrat en métal dur ou carbure cémenté, pour la réception de revêtements en oxyde, résistants, à l'usure, qui comprend:
(a) l'application d'un premier revêtement, sur le substrat, en carbure, nitrure ou carbonitrure de titane, zirconium, hafnium, vanadium, niobium, tantale, chrome, molybdène, tungstène, silicium ou bore;
(b) le traitement du substrat revêtu dans une première atmosphère, choisi parmi les atmosphères formant des carbures et des oxycarbures, pour former une couche de liaison en un carbure ou oxycarbure d'un métal choisi parmi au moins un des tantale, niobium et vanadium, sur ledit substrat revêtu;
(c) le chauffage du substrat revêtu provenant de (b) à une température de 800° à 1300° dans une autre atmosphère oxydante, jusqu'à ce qu'au moins des parties de la surface soient oxydées; et
(d) le traitement du substrat revêtu oxydé provenant de (c) dans une atmosphère réductrice avec un composé réductible de l'aluminium, pour faire diffuser l'aluminium dans le revêtement.

4. Procédé tel que revendiqué dans la revendication 3, comprenant l'étape de superposition d'une couche d'usure en oxyde sur le substrat revêtu oxydé en surface et contenant de l'aluminium.
